# EUROPEAN PATENT SPECIFICATION

(11) **EP 4 638 672 B1**
(45) Date of publication and mention of the grant of the patent: **08.07.2026**
(21) Application number: 23832709.2
(22) Date of filing: 13.12.2023
(51) Int. Cl.: C10M 175/00, C10M 175/02, C10N 20/02, C10N 20/00, C10N 30/02, C10N 30/08, C10N 30/10, C10N 30/00, C10N 40/08, C10N 30/12, C10N 30/18, C10G 21/00

(54) **USE OF RE-REFINED BASE OIL**
VERWENDUNG VON RERAFFINIERTEM BASISÖL
UTILISATION D'HUILE DE BASE RE-RAFFINÉE

(30) Priority: 19.12.2022 CN 202211634787
(43) Date of publication of application: 29.10.2025
(73) Proprietor: Shell Internationale Research Maatschappij B.V., 2596 HR The Hague (NL)
(72) Inventor: NIE, Junfang, Shanghai 201210 (CN); CHEN, Yuan Ting, Shanghai 201210 (CN); SONG, Wei, Houston, Texas 77082-3101 (US)
(74) Representative: Shell Legal Services IP
(86) International application number: PCT/EP2023/085522
(87) International publication number: WO 2024/132751

(56) References cited:
- GURGACZ W ET AL: "PHYSICOCHEMICAL PROPERTIES OF LUBRICATING OIL FRACTIONS OBTAINED BY HYDROREFINING OF WASTE OILS", ERDOEL ERDGAS KOHLE, URBAN VERLAG, HAMBURG, DE, vol. 116, no. 3, 1 March 2000 (2000-03-01), pages 129 - 132, XP000923589, ISSN: 0179-3187
- STIPANOVIC ARTHUR J.: "Compositional Analysis of Re-Refined and Non-Conventional Lubricant Base Oils: Correlations to Sequence VE and IIIE Gasoline Engine Tests", SAE TECHNICAL PAPER 941978, 1 January 1994 (1994-01-01), XP093133660, DOI: 10.4271/941978
- ANONYMOUS: "The rise of re-refining", INSIGHT, 24 August 2021 (2021-08-24), pages 1 - 6, XP093134005, Retrieved from the Internet <URL:https://www.infineuminsight.com/en-gb/articles/the-rise-of-re-refining/> [retrieved on 20240222]

## Description

### Field of the Invention

The present invention relates to the use of re-refined base oils in industrial lubricant oil formulations.

### Background of the Invention

Lubricating fluids are required in all industrial equipment with moving parts. Industrial lubricating fluids, therefore, include hydraulic oils, gear oils, compressor oils, circulating oils and turbine oils, etc. Such industrial lubricating fluids generally comprise one or more base oils and one or more additives. Typically, the additive treat rate for industrial lubricating fluids is considerably lower than for engine oils, with additive treat rates of less than 5wt% being usual.

With such a low additive treat rate, the base oil being used is of key importance. Typically, so called 'virgin' base oils are used in the manufacture of industrial lubricating fluids. These are typically produced from crude oil or natural gas, directly via refining or via synthetic processes.

The disposal of used lubricating fluids requires careful processing and waste streams are often used as burner fuel. In all technology areas, it is necessary to consider the carbon footprint of a product and to try and ensure that raw materials are re-used and recycled where possible. This has led to the development of so called "re-refined base oils". Re-refined base oils (RRBOs) are base oils derived from reprocessing of used lubricating oils to remove contaminants, oxidized products, and additives.

Technologies such as distillation, thermal de-asphalting, or solvent (often propane) de-asphalting are used as recycling technologies for used lubricating fluids. The intermediate products created by recycling technologies are unfinished and typically unsuited for use as lubricants without further improvement. Finishing technologies such as clay treatment, hydrotreatment (see, for example, EP3921390A1, US11034895B1), or solvent extraction (as described in CN107574012A may then be used to "finish" the quality of the intermediates into marketable base oils. When a recycling technology and a finishing technology are coupled together, they are generally referred to as a re-refining technology. A further, pre-treatment, step may also be used to remove sludge, water and additive metals before recycling occurs.

Previously, re-refined base oils have been viewed as inferior in quality to virgin base oils. With the development of improved re-refining technologies this is no longer the case. However, the focus on re-refining technologies and the re-refined base oil thus produced has focused on producing and using base oils of sufficient quality that they can pass the standards set for lubricating oils across industrial technologies (see, for example, CN104673460A and CN104673461A). STIPANOVIC ARTHUR J.: "Compositional Analysis of Re-Refined and Non-Conventional Lubricant Base Oils: Correlations to Sequence VE and IIIE Gasoline Engine Tests",SAE TECHNICAL PAPER 941978, 1 January 1994 (1994-01-01), XP093133660,DOI: 10.4271/941978 discloses the compositional analysis of re-refined and non-conventional lubricant base oils. It is the intention of the present inventors to develop improved lubricating oils using RRBOs.

### Summary of the Invention

The present invention therefore provides the use of a re-refined base oil in an industrial lubricating fluid, said industrial lubricating fluid comprising at least one base oil and at least one additive, in order to improve one or more of oxidation stability and low temperature performance of said industrial lubricating fluid.

### Detailed Description of the Invention

One or more specific embodiments of the present disclosure will be described below. These described embodiments are examples of the presently disclosed techniques. Additionally, in an effort to provide a concise description of these embodiments, not all features of an actual implementation may be described in the specification.

When introducing elements of various embodiments of the present disclosure, the articles "a," "an," and "the" are intended to mean that there are one or more of the elements. The terms "comprising," "including," and "having" are intended to be inclusive and mean that there may be additional elements other than the listed elements. Additionally, it should be understood that references to "one embodiment" or "an embodiment" of the present disclosure are not intended to be interpreted as excluding the existence of additional embodiments that also incorporate the recited features.

The present inventors have surprisingly found that re-refined base oils may be used in order to provide improved fluids for use as industrial lubricating fluids.

Industrial lubricating fluids include, but are not limited to, those used as hydraulic oils, gear oils, compressor oils, circulating oils and turbine oils. An industrial lubricating fluid according to the present invention comprises at least one base oil and at least one additive.

The industrial lubricating fluid preferably comprises at least 95wt% of base oil. According to the invention, of this base oil, at least a portion and up to 100wt% is re-refined base oil. Preferably at least 10wt% of the base oil in the industrial lubricating fluid is re-refined base oil. Depending on the viscosity grades of industrial lubricating fluid, RRBO treat rates could be as high as almost 100% for the light grades of industrial lubricating fluid while heavy virgin base oils might be needed to close the viscosity gap for heavy grades of industrial lubricating fluid.

Base oil in the industrial lubricating fluid that is not re-refined base oil may be any suitable base oil typically used in a lubricating fluid. Specific examples include base oils belonging to Groups I to IV of the API (American Petroleum Institute - see Table 1) base oil categories, which can be used alone or in a mixture.

**Table 1 - API base oil categories**

| Category | Sulfur (%) | | Saturates (%) | Viscosity index |
|---|---|---|---|---|
| Group I | >0.03 | and/or | <90 | 80 - <120 |
| Group II | ≤0.03 | and | ≥90 | 80 - <120 |
| Group III | ≤0.03 | and | ≥90 | ≥120 |
| Group IV | PAO Synthetic Lubricants | | | |
| Group V | All other base oils | | | |

The re-refined base oil used in the present invention is Group I according to the API base oil categories. Typical re-refined Group I base oils, while falling within the API categorisation for Group I base oils have features not typical for a virgin Group I base oil. The saturates content of the Group I re-refined base oil is at least 90%. The viscosity index of the Group I re-refined base oil is at least 95 and preferably at least 105. The sulphur content of the Group I re-refined base oil is no more than 0.3% and preferably no more than 0.1%. The sulphur content of the Group I re-refined base oil is greater than 0.03%, in line with the API classification.

The re-refined base oil use in the present invention is preferably base oil that has been recycled from used lubricant fluid using solvent extraction or hydrotreatment.

Preferably the overall amount of additives in the industrial lubricating fluid is less than 5wt%, more preferably less than 3wt%, even more preferably less than 2wt% based on the overall weight of the industrial lubricating fluid. Suitably, the overall amount of additives in the industrial lubricating fluid is at least 0.1wt% based on the overall weight of the industrial lubricating fluid. The additives may be incorporated into the industrial lubricating fluid singly or as part of one or more additive packages. Whether added singly or in additive packages, a diluent oil may be included with the additive and form part of the finished industrial lubricating fluid.

Different types of additives will be suitable depending on the end use of the industrial lubricating fluid. These include, but are not limited to anti-wear additives, extreme pressure additives, friction modifiers, viscosity index improvers, pour point depressants, antioxidants, rust and corrosion inhibitors, dispersants, demulsifiers and foam inhibitors.

Anti-wear additives and extreme pressure additives include phosphorus compounds, such as phosphate esters, acidic phosphate esters, amine salts of acidic phosphate esters, basic phosphate esters, phosphite esters, phosphorothionates, zinc dithiophosphates, esters of dithiophosphoric acid and alkanols or polyether-type alcohols, and derivatives thereof, phosphorus-containing carboxylic acids and phosphorus-containing carboxylic acid esters.

As examples of viscosity-index improvers mention may be made of non-dispersant type viscosity-index improvers such as polymethacrylates and olefin polymers such as ethylene-propylene copolymers, styrene-diene copolymers, polyisobutylene and polystyrene, and dispersant type viscosity-index improvers where nitrogen-containing monomers have been copolymerised with these, and they may be made with kinds different from the copolymers of olefins and alkyl methacrylates.

As examples of pour-point depressants mention may be made of polymethacrylate-based polymers.

Suitable antioxidants include amine-based antioxidants, sulphur-based antioxidants, phenol-based antioxidants and phosphorus-based antioxidants. These antioxidants may be used singly or in combination.

As examples of demulsifiers suitable for use in industrial lubricating fluids according to this invention, mention may be made of those in the known art normally used as additives for lubricating oils.
Defoaming agents may also be added in order to impart defoaming characteristics to the lubricating oil composition of this invention.

As examples of defoaming agents suitable for use in industrial lubricating fluids according to this invention, mention may be made of organosilicates such as dimethylpolysiloxane, diethylsilicate and fluorosilicone, and non-silicone type defoaming agents such as polyalkylacrylates.

The present invention will now be illustrated through the following, non-limiting examples.

### Examples

A range of industrial lubricant formulation were blended and tested as set out in Tables 3 to 6. The following base oils (with properties as set out in Table 2) were used in the Examples.

The Group I 150SN & 500SN are commercially available from Hindustan Petroleum Corporation Limited (HPCL) under the brand name of Alprol N32 & Alprol N100.

The Group II 150N & 500N are commercially available from Hainan Handi Sunshine Petrochemical Co. under the brand name of HDS-150N & HDS-500N.

The Group I RRBO 150SN is commercially available from Hebei Jingu Recycling Resources Development Co. under the brand name of JINGU 150SN.

The Group II RRBO 150N is commercially available from Changzhou FINAS Energy Technology Co. under the brand name of FINAS 150N.

**Table 2**

| **Properties** | **Test method** | **HPCL 150SN** | **HPCL 500SN** | **HANDI SUNSH INE 150N** | **HAND I SUNSH INE 500N** | **JINGU RRBO 150SN** | **FINAS RRBO 150N** |
|---|---|---|---|---|---|---|---|
| Vk @ 100°C (cSt) | ASTM D445 | 5.293 | 10.67 | 5.386 | 10.13 | 5.492 | 5.318 |
| Vk @ 40°C (cSt) | ASTM D445 | 31.56 | 93.54 | 31.54 | 82.61 | 31.27 | 28.97 |
| Viscosity Index | ASTM D2270 | 98 | 97 | 104 | 103 | 112 | 118 |
| Saturates (%) | IP 368/ASTM D7419 | 74.4 | 61.5 | 99.8 | 99.8 | 96.6 | 97 |
| Sulphur content (%) | ASTM D5453 | 0.97 | 1.38 | 0.000 1 | 0.000 2 | 0.047 7 | 0.007 7 |

The hydraulic oil package used in the formulations is a commercially available standard industrial hydraulic oil additive package.

The pour point depressant used in the formulations is a standard, commercially available, pour point depressant.

The anti-foam additive used in the formulations is a commercially available anti-foam additive.

It can be seen from Tables 3 to 6 that Group I or Group II RRBO based samples show performance advantages, against their virgin base oil counterparts, like higher VI, lower viscosity at 0°C, better oxidation stability as reflected by RPVOT and TOST test outcomes.

**Table 3 (Ex 2 for reference)**

| | | **Comp Ex. 1** | **Comp Ex. 2** | **Ex 1** | **Ex 2** |
|---|---|---|---|---|---|
| Group I 150SN | | 89.5 | | | |
| Group I 500SN | | 9.94 | | | |
| Group II 150N | | | 95.47 | | |
| Group II 500N | | | 3. 97 | 6.34 | 11.79 |
| Group I RRBO 150SN | | | | 92.7 | |
| Group II RRBO 150N | | | | | 87.7 |
| Hydraulic oil package 1 | | 0.45 | 0.45 | 0.45 | 0.45 |
| Pour point depressant 2 | | 0.1 | 0.1 | 0.5 | 0.05 |
| Anti-foam additive 3 | | 0.01 | 0.01 | 0.01 | 0.01 |

| **Properties** | **Test method** | | | | |
|---|---|---|---|---|---|
| Appearance | Visual | B&C | B&C | B&C | B&C |
| Vk @ 40°C (cSt) | GB/T 265 | 35.27 | 34.31 | 33.63 | 32.76 |
| Vk @ 100°C (cSt) | GB/T 265 | 5.751 | 5.760 | 5.843 | 5.762 |
| Viscosity Index | GB/T 1995 | 103 | 108 | 117 | 118 |
| Vk @ 0°C (cSt) | GB/T 265 | 383.0 | 346.3 | 317.3 | 304.7 |
| Copper, 3 h, 100°C | GB/T 5096 | 1b | 1b | 1a | 1a |
| Rust, SSW, Method B - 24 Hours | GB/T 11143 | No Rustin g | No Rustin g | No Rustin g | No Rustin g |
| Foaming Seq I, ml.ml | GB/T 12579 | 0/0 | 30/0 | 10/0 | 50/0 |
| Seq II, ml/ml | | 30/0 | 10/0 | 10/0 | 30/0 |
| Seq III, ml/ml | | 0/0 | 0/0 | 10/0 | 50/0 |
| water separation @ 54°C | GB/T 7305 | 25 | 20 | 10 | 10 |
| TOST Oxidation Stability | GB/T 12581 | | | | |
| Total acid number after 1000hrs | | 0.3 | 0.24 | 0.093 | 0.12 |
| RPVOT, 150°C (min) | SH/T 0193 | 205 | 212 | 265 | 228 |
| Filterability (Stage I)-Dry (%) | ISO 13357-2: 2017 | 84.7 | 88.6 | 96.3 | 94.2 |
| Filterability (Stage II)-Dry (%) | | 67.0 | 78.6 | 94.7 | 90.1 |
| Filterability (Stage I)-Wet | ISO 13357-1: 2017 | 91.9 | 78.3 | 87.0 | 82.0 |
| Filterability (Stage II)-Wet | | 83.9 | 54.9 | 79.0 | 64.0 |

**Table 4 (Ex 4 for reference)**

| | | **Comp Ex.3** | **Comp Ex. 4** | **Ex 3** | **Ex 4** |
|---|---|---|---|---|---|
| Group I 150SN | | 29.83 | | | |
| Group I 500SN | | 69.61 | | | |
| Group II 150N | | | 14. 92 | | |
| Group II 500N | | | 84.52 | 69.04 | 74.49 |
| Group I RRBO 150SN | | | | 30 | |
| Group II RRBO 150N | | | | | 25 |
| Hydraulic oil package 1 | | 0.45 | 0.45 | 0.45 | 0.45 |
| Pour point depressant 2 | | 0.1 | 0.1 | 0.5 | 0.05 |
| Anti-foam additive 3 | | 0.01 | 0.01 | 0.01 | 0.01 |

| **Properties** | **Test method** | | | | |
|---|---|---|---|---|---|
| Appearance | Visual | B&C | B&C | B&C | B&C |
| Vk @ 40°C (cSt) | GB/T 265 | 67.2 | 68.31 | 65.92 | 68.01 |
| Vk @ 100°C (cSt) | GB/T 265 | 8.631 | 9.060 | 8.992 | 9.109 |
| Viscosity Index | GB/T 1995 | 99 | 107 | 111 | 109 |
| Vk @ 0°C (cSt) | GB/T 265 | 957.6 | 938.3 | 826.9 | 916.0 |
| Copper, 3 h, 100°C | GB/T 5096 | 1b | 1b | 1a | 1a |
| Rust, SSW, Method B - 24 Hours | GB/T 11143 | No Rustin g | No Rustin g | No Rustin g | No Rustin g |
| Foaming Seq I, ml.ml | GB/T 12579 | 0/0 | 60/0 | 10/0 | 0/0 |
| Seq II, ml/ml | | 60/0 | 30/0 | 20/0 | 30/0 |
| Seq III, ml/ml | | 0/0 | 0/0 | 10/0 | 0/0 |
| water separation @ 54°C | GB/T 7305 | 30 | 20 | 15 | 10 |
| TOST Oxidation Stability | GB/T 12581 | | | | |
| Total acid number after 1000hrs | | 0.25 | 0.19 | 0.10 | 0.17 |
| RPVOT, 150°C (min) | SH/T 0193 | 173 | 215 | 202 | 208 |
| Filterability (Stage I)-Dry (?s) | ISO 13357-2: 2017 | 82.7 | 93.1 | 93.3 | 85 |
| Filterability (Stage II)-Dry (%) | | 65.7 | 86.0 | 86.5 | 74.5 |
| Filterability (Stage I)-Wet | ISO 13357-1:2017 | 92.5 | 80.5 | 88.0 | 83 |
| Filterability (Stage II)-Wet | | 84.1 | 61.2 | 80.0 | 74 |

**Table 5 (Ex 6 for reference)**

| | | **Example 5** | **Example 6** |
|---|---|---|---|
| Group I 150SN | | | |
| Group I 500SN | | | |
| Group II 150N | | | |
| Group II 500N | | 39.96 | 43.41 |
| Group I RRBO 150SN | | 59.08 | |
| Group II RRBO 150N | | | 56.08 |
| Hydraulic oil package 1 | | 0.45 | 0.45 |
| Pour point depressant 2 | | 0.5 | 0.05 |
| Anti-foam additive 3 | | 0.01 | 0.01 |

| **Properties** | **Test method** | | |
|---|---|---|---|
| Appearance | Visual | B&C | B&C |
| Vk @ 40°C (cSt) | GB/T 265 | 46.51 | 46. 68 |
| Vk @ 100°C (cSt) | GB/T 265 | 7.170 | 7.204 |
| Viscosity Index | GB/T 1995 | 114 | 114 |
| Vk @ 0°C (cSt) | GB/T 265 | 517.9 | 509.2 |
| Copper, 3 h, 100°C | GB/T 5096 | 1a | 1a |
| Rust, SSW, Method B - 24 Hours | GB/T 11143 | No Rusting | No Rusting |
| Foaming Seq I, ml/ml | GB/T 12579 | 10/0 | 0/0 |
| Seq II, ml/ml | | 10/0 | 30/0 |
| Seq III, ml/ml | | 10/0 | 0/0 |
| water separation @ 54°C | GB/T 7305 | 10 | 10 |
| TOST Oxidation Stability | GB/T 12581 | | |
| Total acid number after 1000hrs *mg KOH/g | | 0. 089 | 0.11 |
| RPVOT, 150°C (min) | SH/T 0193 | 226 | 267 |
| Filterability (Stage I)-Dry (%) | ISO 13357-2:2017 | 96.5 | 87.5 |
| Filterability (Stage II)-Dry (%) | | 93.1 | 76.6 |
| Filterability (Stage I)-Wet | ISO 13357-1:2017 | 86 | 78 |
| Filterability (Stage II)-Wet | | 76 | 58 |

**Table 6**

| | | **Comp Ex. 5** | **Comp Ex 6** | **Example 7** |
|---|---|---|---|---|
| Group I 150SN | | 64.41 | | |
| Group I 500SN | | 34.63 | | 36.67 |
| Group II 150N | | | 59.7 | |
| Group II 500N | | | 39.79 | |
| Group I RRBO 150SN | | | | 62.37 |
| Group II RRBO 150N | | | | |
| Hydraulic oil package 1 | | 0.45 | 0.45 | 0.45 |
| Pour point depressant 2 | | 0.5 | 0.05 | 0.5 |
| Anti-foam additive 3 | | 0.01 | 0.01 | 0.01 |

| **Properties** | **Test method** | | | |
|---|---|---|---|---|
| Appearance | Visual | B&C | B&C | B&C |
| Vk @ 40°C (cSt) | GB/T 265 | 46.20 | 45.11 | 46.52 |
| Vk @ 100°C (cSt) | GB/T 265 | 6.710 | 6.869 | 6.850 |
| Viscosity Index | GB/T 1995 | 97 | 108 | 102 |
| Vk @ 0°C (cSt) | GB/T 265 | 558.2 | 510.3 | 520.4 |
| Copper, 3 h, 100°C | GB/T 5096 | 1a | 1a | 1a |
| Rust, SSW, Method B - 24 Hours | GB/T 11143 | No Rusting | No Rusting | No Rusting |
| Foaming Seq I, ml/ml | GB/T 12579 | 0/0 | 0/0 | 0/0 |
| Seq II, ml/ml | | 10/0 | 20/0 | 10/0 |
| Seq III, ml/ml | | 0/0 | 0/0 | 0/0 |
| water separation @ 54°C | GB/T 7305 | 30 | 10 | 25 |
| TOST Oxidation Stability | GB/T 12581 | | | |
| Total acid number after 1000hrs *mg KOH/g | | 0.64 | 0.22 | 0.11 |
| RPVOT, 150°C (min) | SH/T 0193 | 192 | 216 | 244 |
| Filterability (Stage I)-Dry (%) | ISO 13357-2:2017 | 95.8 | 94.6 | 96.3 |
| Filterability (Stage II)-Dry (%) | | 92.3 | 90.4 | 92.6 |
| Filterability (Stage I)-Wet | ISO 13357-1:2017 | 64 | 82 | 88 |
| Filterability (Stage II)-Wet | | 20 | 67 | 74 |

## Claims

1. Use of a re-refined base oil in an industrial lubricating fluid, said industrial lubricating fluid comprising at least one base oil and at least one additive, in order to improve one or more of oxidation stability and low temperature performance of said industrial lubricating fluid, wherein the re-refined base oil is a Group I base oil with a viscosity index of at least 95, a sulphur content of no more than 0.3% measured according to ASTM D5453 and a saturates content of at least 90% measured according to IP 368 / ASTM D7419.

2. Use according to Claim 1, wherein the industrial lubricating fluid comprises at least 95wt% of base oil.

3. Use according to Claim 1 or Claim 2, wherein at least a portion and up to 100wt% of the base oil is re-refined base oil.

4. Use according to any one of Claims 1 to 3, the re-refined base oil is base oil that has been recycled from used lubricant fluid using solvent extraction or hydrotreatment.

5. Use according to any one of Claims 1 to 4, wherein the overall amount of additives in the industrial lubricating fluid is less than 5wt%, more preferably less than 3wt%, even more preferably less than 2wt% based on the overall weight of the industrial lubricating fluid.

## Patentansprüche

1. Verwendung eines wiederaufbereiteten Grundöls in einem industriellen Schmierfluid, wobei das industrielle Schmierfluid mindestens ein Grundöl und mindestens einen Zusatzstoff umfasst, um eines oder mehrere von Oxidationsstabilität und Tieftemperaturverhalten des industriellen Schmierfluids zu verbessern, wobei das wiederaufbereitete Grundöl ein Gruppe-I-Grundöl mit einem Viskositätsindex von mindestens 95, einem Schwefelgehalt von höchstens 0,3 %, gemessen nach ASTM D5453, und einem Sättigungsgehalt von mindestens 90 %, gemessen nach IP 368 / ASTM D7419, ist.

2. Verwendung nach Anspruch 1, wobei das industrielle Schmierfluid mindestens 95 Gew.-% Grundöl umfasst.

3. Verwendung nach Anspruch 1 oder Anspruch 2, wobei mindestens ein Teil und bis zu 100 Gew.-% des Grundöls wiederaufbereitetes Grundöl ist.

4. Verwendung nach einem der Ansprüche 1 bis 3, wobei das wiederaufbereitete Grundöl ein Grundöl ist, das aus gebrauchtem Schmiermittelfluid unter Verwendung von Lösungsmittelextraktion oder Hydrobehandlung recycelt wurde.

5. Verwendung nach einem der Ansprüche 1 bis 4, wobei die Gesamtmenge an Zusatzstoffen in dem industriellen Schmierfluid weniger als 5 Gew.-%, mehr bevorzugt weniger als 3 Gew.-%, noch mehr bevorzugt weniger als 2 Gew.-%, bezogen auf das Gesamtgewicht des industriellen Schmierfluids, beträgt.

## Revendications

1. Utilisation d'une huile de base reraffinée dans un fluide de lubrification industrielle, ledit fluide de lubrification industrielle comprenant au moins une huile de base et au moins un additif, afin d'améliorer une ou plusieurs parmi une stabilité à l'oxydation et des performances à basse température dudit fluide de lubrification industrielle, dans laquelle l'huile de base reraffinée est un groupe I une huile de base avec un indice de viscosité d'au moins 95, une teneur en soufre ne dépassant pas 0,3 % mesurée selon la norme ASTM D5453 et une teneur en composés saturés d'au moins 90 % mesurée selon la norme IP 368/ASTM D7419.

2. Utilisation selon la revendication 1, dans laquelle le fluide lubrifiant industriel comprend au moins 95 % en poids d'huile de base.

3. Utilisation selon la revendication 1 ou la revendication 2, dans laquelle au moins une partie et jusqu'à 100 % en poids de l'huile de base est de l'huile de base reraffinée.

4. Utilisation selon l'une quelconque des revendications 1 à 3, l'huile de base reraffinée est une huile de base qui a été recyclée à partir d'un fluide lubrifiant usagé par extraction par solvant ou hydrotraitement.

5. Utilisation selon l'une quelconque des revendications 1 à 4, dans laquelle la quantité globale d'additifs dans le fluide lubrifiant industriel est inférieure à 5 % en poids, plus préférablement inférieure à 3 % en poids, encore plus préférablement inférieure à 2 % en poids sur la base du poids global du fluide lubrifiant industriel.
